

## UNITED STATES PATENT OFFICE

1,984,214

## PROCESS FOR THE LUBRICATION OF SURFACES WHICH ARE EXPOSED TO A HIGH TEMPERATURE

Moritz Joseph Heitmann, Freital, Germany, assignor, by mesne assignments, to The Patent and Licensing Corporation, New York, N. Y., a corporation of Massachusetts

No Drawing. Application September 18, 1929,  
Serial No. 393,581

## 3 Claims. (Cl. 87—9)

This invention concerns a process for the lubrication, of hot moving surfaces as for example, bearings which are exposed to high temperatures.

Bearings which are exposed to high temperatures occur, for instance, in rolling mills used in the manufacture of iron plates and the like. The lubrication of these bearings, which some times may attain temperatures of 300 to 400° C., or even higher, offers great difficulties. As is known, the lubricants which are ordinarily used, such as mineral oils, vegetable oils, fats and the like, cannot exert a sufficient lubricating action at these high temperatures. Therefore, other lubricants have been proposed which are able to form lubricating films at these temperatures. Such substances are, for instance, the residue of distillation of mineral oils, such as asphalt. The application of these materials, however, offers many difficulties mainly due to the high viscosity of these products at normal temperatures, resulting in the impossibility of conveying these lubricants to the parts to be lubricated, in the ordinary way. It has been attempted to avoid these difficulties by adding so-called flux to the asphalt, but then another difficulty arises, namely: the danger of the lubricant taking fire from the high temperature of the bearings, which temperature is generally higher than the flash point of the flux. Another method has been attempted consisting in conveying the lubricant at an elevated temperature so as to assure viscosity which is sufficiently low to permit the use of devices ordinarily used when applying lubricants of a low viscosity.

This invention avoids the difficulties by the use of a lubricant consisting of bituminous material such as asphalt, in an emulsified condition. The asphalt, the properties of which must be chosen in accordance with the circumstances at the place to be lubricated, forms the dispersed phase of the emulsion while the dispersing phase of the emulsion comprises water. The preparation of the emulsions may take place in any known manner. So, for instance, the emulsion can be made by mixing the asphalt containing a small amount of an acid soluble therein such as napthenic acid, sulphonic acid, oleic acid, or the like, with the aqueous phase containing a suitable concentration of an alkaline substance such as NaOH, KOH, Na<sub>2</sub>CO<sub>3</sub>, or the like. Again, the asphalt can be emulsified in the dispersing phase containing a suitable amount of an emulsifier or stabilizer such as soap, albumin, clay, or the like, with the help of a colloid mill or other convenient form of emulsifying apparatus. The so obtained emulsion may be further stabilized in any known manner in

order to impart the required stability against storage, transport, freezing and the like, by the addition of a suitable amount of a stabilizer such as albumins, saponin, casein, tannin, and the like.

In the use of the emulsion for lubricating hot bearings of the type indicated, the emulsion can be fed continuously to the bearings from a convenient storage tank. This provides an advantageous operating condition over the present practice wherein hot asphalt is used for this purpose, in which case it is generally necessary for the operator to daub the bearings from time to time with a hand operation. With the use of the emulsion, the obvious difficulties attendant upon the aforescribed hand operation are eliminated, since any suitable feed mechanism adopted for continuously feeding as by gravity or pumping, a stream of emulsion to the bearings may be employed.

Upon reaching the bearings, the water contained in the emulsion, being in the continuous phase, evaporates rather quickly and almost instantaneously, in as much as the temperature of the bearings is as high as 300 to 400° C. and the bearings themselves are generally of an open type construction permitting evolution of the steam formed from the water. In any event, however, the presence of the water does not interfere with the lubricating value of the asphalt contained in the dispersed phase of the emulsion, and in fact, the presence of the water is advantageous due to the additional cooling effect of the water. Upon the evaporation of water, however, there is left in the bearing asphalt in molten condition, forming a lubricating film around the bearing in much the same manner as when using hot asphalt as such, but without the difficulties that normally prevail in the application of hot asphalt to the bearings.

The emulsion used may comprise 20 to 60% of asphalt in the dispersed phase, the actual concentration of asphalt, however, being governed by the temperature of the bearings and the viscosity of the emulsion, which must be low enough to permit an even and continuous feed thereof to the bearings. When it is required to realize a considerable cooling effect from the water of the emulsion, the latter may be more dilute, that is to say, it should contain less asphalt in proportion to the water content thereof.

The use of asphalt in aqueous emulsified condition presents an additional advantage in that the lubricating effect may be substantially increased by combining with the prepared emulsion, or with the water prior to emulsification, or in some in-

stances, with the asphalt prior to emulsification, substances such as graphite in finely divided form. If this be attempted when using hot asphalt as a lubricant, the viscosity of the molten asphalt is further increased by the graphite, thus further increasing the difficulties in handling, whereas in accordance with the invention, any increase in viscosity of the emulsion due to introduction of graphite or the like, may be readily compensated by reducing the viscosity with additional quantities of water, or by a further beating action.

I claim as my invention:

1. The process of lubricating surfaces exposed

to high temperatures comprising applying to said surfaces an aqueous dispersion of highly viscous bitumen.

2. The process of lubricating surfaces exposed to high temperatures comprising applying to said surfaces an aqueous dispersion of asphalt.

3. The process of lubricating surfaces exposed to high temperatures comprising applying to said surfaces an aqueous dispersion of asphalt containing a finely divided solid lubricant.

5

10

MORITZ JOSEPH HEITMANN.